

# UNITED STATES PATENT OFFICE.

ARTHUR EICHENGRÜN, OF BERLIN, GERMANY.

## PLASTIC COMPOSITION.

1,185,074.

Specification of Letters Patent.

Patented May 30, 1916.

No Drawing.

Application filed August 1, 1910. Serial No. 574,969.

*To all whom it may concern:*

Be it known that I, ARTHUR EICHENGRÜN, Ph. D., of 87 Konstanzerstrasse, Berlin, in the Kingdom of Prussia and German Empire, have invented new and useful Improvements in Plastic Compositions.

Whereas it is possible to mix with celluloid made from nitro-cellulose 20-25% of filling material, such as, for instance, zinc white, without affecting the celluloid character and especially the tenacity of the material, this has not yet been possible in the case of acetyl cellulose. Apart from the fact that hitherto it was only possible to produce a plastic, pliable material, but not a solid celluloid-like material from acetyl cellulose in thick sheets or plates, an admixture of filling materials also acted very unfavorably upon the thin celluloid-like sheets remaining after evaporation of solutions of acetyl cellulose containing camphor or camphor substitutes, since the addition of even less than 25% of filling materials rendered these sheets brittle.

Now it has been found possible to obtain from acetyl cellulose and filling materials a new material having very valuable technical properties, by adding to the acetyl cellulose a larger amount of camphor substitutes than is necessary for producing the celluloid-like character, or by replacing the camphor substitutes proper with softening admixtures and then adding not only 20-25% of filling materials, as is the case with celluloid, but larger amounts of same. In this process the excessive plasticity and ductility produced by the camphor substitutes or the softening admixtures is compensated by the amount of the hardening filling materials, and a new product is produced which is essentially different from celluloid mixed with filling materials. Whereas namely, it is only at temperatures over 100 degrees centigrade that the latter softens sufficiently to be capable of being pressed in molds, blown or stamped, the new material already softens at about 75 degrees centigrade. Whereas celluloid plates or sheets have to be cooled while under pressure and must be cooled directly after molding, the new material retains, without further treatment, the form given to it while hot.

While celluloid, especially in making molded or pressed articles, must be submitted to very high pressure, for instance, in a lever press, the new material can be

worked under very slight pressure, and nevertheless shows the details of the mold more clearly than the highly heated celluloid molded under high pressure.

A further advantage of the new material consists in the low cost of production. Whereas with celluloid, as mentioned above, only a fraction of its own weight of filling material can be added, acetyl cellulose in the presence of softening admixtures can easily be mixed with twice or even four times its own amount of filling material without making the mass brittle, consequently the cost of production of the latter is several times less than that of acetyl cellulose.

I will explain my process by means of the following example: One kilo acetyl cellulose is mixed with 300 grams acetyl methyl anilid and 300 grams of ethylester of lactic acid, one kilo alcohol and one kilo of benzene is added and the whole heated to 70 degrees centigrade. After solution 2 kilos zinc white are admixed and the resulting viscous mass is poured out onto a flat surface. The mass solidifies at once to a homogeneous sheet or plate, which when quite dry assumes the form of a solid celluloid-like material of great plasticity, and possessing the afore-mentioned properties.

Instead of the mixture mentioned, cold-acting solvents may be employed, the troublesome formation of bubbles during the evaporation of acetyl cellulose solutions being prevented by the presence of the large amount of filling material, and thick homogeneous plates also can be produced by means of easily volatile solutions such as acetone. In the same manner the filling material can be worked directly with the acetate and the admixtures with or without the presence of solvents, into a homogeneous mass, by kneading while hot, and if desired under pressure, in this case because the excessive softening action of the quantity of admixtures required for the production of such a mass is counteracted by the amount of the filling material. Finely powdered substances of all kinds, such as mineral-, metal-, vegetable powders, graphite, lamp black and the like, can be employed as filling materials.

The amount of the softening admixture or camphor substitute required depends on the nature of the filling material used and also upon the character of the final material which is to be obtained. When speaking of

the final character of the material to be obtained I do not refer to the solid mass nor the celluloid-like character but to various other characteristics or qualities which it is desirable to impart to the material according to the use for which it is required.

It should be noted that, with the present process, the rigidity or hardness of the material prepared from acetyl cellulose and admixtures, which is too soft without filling materials, is essentially increased by admixing the latter in large amounts, and that a hard and celluloid-like material is produced which only becomes plastic when heated, possesses great commercial value and has proved to be applicable to a large field of uses for which hitherto rubber, celluloid, soft metal or the like have been employed, as for instance for the production of packing material, electric insulating material, heat insulating and the like materials. The new mass can further be used for the production of piano keys, hollow bodies, receptacles, hoods and coverings, or platings for wood, metal, paper and the like foundations, or the material may be blown into the shape of dolls, animals and the like toys.

What I claim as new and desire to secure by Letters Patent is:—

30 1. A composition of matter consisting of

a celluloid-like material which at an ordinary or room temperature is perfectly hard but is capable when heated of being blown and worked into articles of use comprising acetyl cellulose together with filling materials in quantities essentially over 25 per cent. of the weight of the acetyl cellulose, there being incorporated with the mass as much of softening admixtures as is required by the nature of the filling material 40 employed.

2. A composition of matter consisting of a celluloid-like material which at an ordinary or room temperature is perfectly hard but is capable when heated of being blown 45 and worked into articles of use comprising acetyl cellulose together with filling materials in quantities essentially over 100 per cent. of the weight of the acetyl cellulose, there being incorporated with the mass as 50 much of softening admixtures as is required by the nature of the filling material employed.

In testimony, that I claim the foregoing as my invention, I have signed my name in presence of two subscribing witnesses.

ARTHUR EICHENGRÜN.

Witnesses:

WALDEMAR HAUPT,  
HENRY HASPER.